

ENTIMENT & CHEMICAL MODIFI-  
CATION OF TEXTILES & FIBERS,

## UNITED STATES PATENT OFFICE.

FREDERICK EUGENE DROWN, OF PAWTUCKET, RHODE ISLAND.

## PROCESS OF BLEACHING COTTON.

SPECIFICATION forming part of Letters Patent No. 396,551, dated January 22, 1889.

Application filed May 2, 1888. Serial No. 272,596. (No specimens.)

*To all whom it may concern:*

Be it known that I, FREDERICK EUGENE DROWN, a citizen of the United States, residing at Pawtucket, in the county of Providence and State of Rhode Island, have invented a new and useful Process of Bleaching Cotton Fabrics, of which the following is a specification.

The object of my invention is to bleach cotton fabric expeditiously without materially reducing its strength.

In my application for a patent filed March 19, 1888, Serial No. 267,707, I have described means of treating with caustic soda, soda-ash, or lime, and the washing, chemicing, and souring of cotton fabric in an improved keir having a centrifugal basket inclosed in a vessel which at times can be made steam-tight.

My present invention consists of the following successive steps of operation: I pass the cotton fabric, spread out to its full width and in a continuous manner, through a hot solution of caustic soda having a strength of from 6° to 12° Twaddle; thence through heavy squeezing-rolls, then subjecting it to the action of steam by passing it over perforated steam-pipe in an open vessel where the temperature cannot exceed 212° Fahrenheit; thence into a cold solution of caustic soda having a strength of 6° to 12° Twaddle and a temperature of not over 110° Fahrenheit; thence through heavy squeezing-rolls. I run the cloth during this step of the process continuously at a speed of sixty to one hundred yards per minute. I then run the cotton fabric into the bleaching-keir. I find the keir as described in my application for a patent above referred to very effective, and subject

it to a continuously-extracting circulation of a boiling solution of soda-ash and rosin in a closed vessel, about twenty-five pounds of refined soda-ash and ten pounds of rosin to one ton of cotton fabric. This treatment is continued for several hours until the motes are decomposed or destroyed, when I wash the cotton fabric with hot water of not less than 140° Fahrenheit. The cotton fabric is then treated with chlorine liquor having a strength of two-tenths of 1° Twaddle. Then I subject it to the action of steam in an open vessel, where the temperature cannot exceed 212° Fahrenheit. The cotton fabric is then soured, the liquor to be 100° to 110° Fahrenheit and having a strength of two-tenths of 1° Twaddle when at a temperature of 75° Fahrenheit. The fabric is now washed.

Having thus described my invention and the manner of carrying it out in practice, I claim as my invention and desire to secure by Letters Patent—

The improvement in the art of bleaching, consisting in passing cotton fabric spread out wide through a boiling solution of caustic soda, then subjecting it to the action of steam by passing it over perforated steam-pipe, then cooling it by passing it into a cold solution of caustic soda, then boiling in a solution of soda-ash and washing, then subjecting the material to the action of chlorine liquor, then steaming, souring, and finally washing, substantially as set forth.

FREDERICK EUGENE DROWN.

Witnesses:

SAMUEL B. LORD,  
CHARLES W. LORD.